

June 11, 1968

C. E. JACKSON ET AL

3,388,200

PROCESS FOR WET SPINNING ELASTIC FIBERS

Filed Dec. 21, 1964



FIG. 1.



FIG. 2.

INVENTORS

CHARLES E. JACKSON  
LLOYD T. JENKINS  
PHILIP E. SLADE, JR.

BY *O. Weller Connell Jr.*  
ATTORNEY

1

3,388,200

PROCESS FOR WET SPINNING ELASTIC FIBERS  
Charles E. Jackson, Durham, Lloyd T. Jenkins, Cary,  
and Philip E. Slade, Jr., Chapel Hill, N.C., assignors to  
Monsanto Company, St. Louis, Mo., a corporation of  
Delaware

Filed Dec. 21, 1964, Ser. No. 419,779  
5 Claims. (Cl. 264—184)

## ABSTRACT OF THE DISCLOSURE

The wet spinning of linear, fiber-forming, segmented polyurethane polymers is improved by positioning the spinneret so that the fiber rises vertically from the spinneret and remains in the coagulation bath for only about 0.2 seconds or less. The fiber has greater elongation than by prior wet spinning methods and retains good tenacity.

This invention relates to the preparation of shaped articles from linear, segmented polyurethane compositions and more particularly to an improved wet spinning method for the preparation of elastic fibers and filaments from linear, segmented, polyurethane polymers typified structurally by the presence of low-melting, amorphous segments joined to high-melting, crystalline segments.

Certain synthetic elastomers based on linear, segmented polyurethane polymers have been developed as a replacement for rubber, which possesses some disadvantages for textile applications that tend to offset its desirable elastic properties. Fibers from these new synthetic elastomers are highly elastic and also have a higher modulus and better abrasion resistance than rubber. It is desirable therefore, to have available a wet spinning process for the preparation of fibers and filaments from these synthetic elastomers which would have a relatively wide range of tenacities, elongations, moduli and other properties which are easily obtained in a controlled and consistently reproducible manner.

It is an object of this invention to prepare elastic fibers and filaments from linear, segmented polyurethane polymers by an improved wet spinning process.

Another object of the invention is to provide a wet spinning process for the preparation of elastic fibers and filaments from linear, segmented polyurethane compositions in which the process is characterized by faster production rates, by the fibers remaining in the spin bath a very short period of time, approximately from about 0.025 to 0.2 second, and by the positioning of the spinneret so that the fiber leaves the spin bath at right angles to the surfaces of the spin bath and travels in an essentially vertical path upwardly to the first godet.

An additional object of the invention is to provide a wet spinning process which produces elastic polyurethane fibers of improved elongation, tenacity, modulus and stress retention.

Yet another object of the invention is to provide a wet spinning process for the preparation of fibers from linear, segmented polyurethane compositions in which the spinneret is immersed only from about 0.5 to 3.0 inches beneath the surface of the coagulation bath and in which the elimination of substantially all friction points in the bath and on the first godet has taken place.

Other objects and advantages of the invention will become apparent from the description which follows:

Wet spinning of fiber-forming polymers wherein the polymer is extruded in a vertical upward direction with short spinneret immersion is well known in viscose spinning art. However, since viscose polymers are composed of regenerated naturally occurring cellulose rather than purely synthetic substances, the spinning conditions in

2

viscose spinning differ radically from those in the case of wet spinning of synthetic polymers. In viscose spinning inorganic salts must be present in the coagulation bath for successful spinning of viscose dopes which contain 5-7% solids. The prior art on wet spinning of linear, segmented polyurethane polymers, as typified by U.S. Patents 2,755,266; 2,923,598; 2,955,07; and 2,965,437, teaches the necessity of having to use long coagulation baths and lengthy immersion time with the spinneret positioned for substantially horizontal extrusion or "horizontal spinning" regardless of whether the polymer is formed prior to spinning or "extended" in the coagulation bath.

It has unexpectedly been found that the wet spinning of linear, segmented polyurethane polymers can be substantially improved by a process which is referred to herein as "vertical spinning" and may generally be described as consisting of extruding a solution of a linear, segmented polyurethane in an organic solvent into an essentially aqueous coagulation bath, withdrawing the filaments as they are coagulated upwardly through the coagulating bath a distance of from about 0.5 to 3.0 inches at a rate of withdrawal which will result in the filaments remaining in the coagulating bath for an immersion time of from only 0.025 to 0.2 second and collecting the filaments for further processing after their emergency from the coagulating bath.

The extrusion of the linear, segmented polyurethane polymer solution may be accomplished by employing a suitable extrusion orifice well known in the art and which is suitable for the preparation of the type of end product desired. The solution of the polymer may be prepared by employing any well known prior art solvent which will dissolve a linear, segmented polyurethane polymer in the desired concentration for spinning, usually from 15-25% solids concentration. Such solvents, for example, include dimethylformamide, dimethylacetamide, dimethylsulfoxide and hexamethylphosphoramide. The preferred solvents are dimethylformamide and dimethylacetamide.

The coagulating bath preferably consists primarily of water at a temperature of from about 60 to 90° C. The coagulating bath may contain a percentage of the organic solvent used to prepare the solution, for example from about 1 to 40 percent.

The positioning of the spinneret beneath the surface of the coagulating bath and the residence time of the fiber in the bath are critical features of the invention. The improvement obtainable in the wet spinning of linear, segmented polyurethane polymers is achieved by placing the spinneret in a position in the coagulating bath so that the filaments as they are extruded out of the spinneret are conveyed in an essentially vertical upward direction through the coagulating bath liquid for a distance of from about 0.5 to 3.0 inches, preferably 1.5 to 2.0 inches and at a rate of withdrawal which will result in the filaments remaining in the coagulating bath for a period of time of from about 0.025 to 0.2 second and preferably from about 0.075 to 0.1 second. Surprisingly, this very short coagulation bath exposure or residence time has been found to be advantageous in effecting coagulation and to do so without void formation. The vertical withdrawal of the filaments reduces solvent drag which is prevalent during normal wet spinning processes wherein a certain amount of the coagulating bath liquid and the spinning solvent is withdrawn partially from the surface of the coagulating bath by the moving filament and then falls back into the coagulating bath. This sets up a certain amount of drag or frictional pull on the filaments as they emerge from the coagulating bath liquid and results in deterioration of critical fiber properties. As a further means for reducing all frictional pull on

the filaments during this soft stage of their development the first godet or roller around which the filaments are wrapped and removed from the coagulating bath is constructed so as to freely rotate or be driven by motor means so that no frictional pull is placed upon the filaments at this point.

Reference will now be made to the appended drawings, in which:

FIGURE 1 is a side elevational view partly in section showing schematically an apparatus arrangement of the type which can be used in carrying out the process of the invention.

FIGURE 2 is a graph showing the effect of residence time and immersion length on elongation, a critical property for elastic fibers.

Referring now in detail to FIGURE 1, a solution of a linear, segmented polyurethane polymer dissolved in an organic solvent is passed under pressure from a supply tank (not shown) by pump 1 through pipe 2 leading into the coagulating bath 3 containing an aqueous coagulating liquid 4. Then the solution is extruded through spinneret 5 in a vertical direction to form filaments 6 which are collected on advancing roller 7 and then forwarded for further suitable fiber conditioning treatments. The solu-

5 extension of the fibers at the breaking point. "Stress retention" is the percent elasticity retained after 300% extension and 80% recovery of the 2nd cycle stretch.

#### EXAMPLE I

To a reactor vessel is added 2,000 parts by weight of a polycaprolactone of molecular weight 2,850, 356 parts of 4,4'-methylenediphenyl diisocyanate in 1,260 parts dimethylformamide solvent. The reaction is allowed to continue for 1.0 to 1.5 hours. At the end of this period the "prepolymer" which results is added to a solution of 41.3 parts of ethylene diamine in 12,340 parts of dimethylformamide to give a spinning dope of 15 percent solids.

10 The spinning dope is extruded through a spinneret containing 15 holes of 6 mil diameter into a coagulation bath containing various amounts of solvent and water at a temperature of 70° C. Residence time, the time the filaments remain in the bath, varied from 2 to 0.75 seconds. All fiber samples were washed, dried, and taken up at a speed of 100 feet per minute. Properties of various fiber samples using both horizontal and vertical spinneret positioning and showing the improvement in elongation obtained with short residence time and vertical spinning are summarized in Table I.

TABLE I

| Experiment No. | Spinneret Direction | Time in Spin Bath (sec.) | Bath Composition   | Denier | Tenacity | Elongation |
|----------------|---------------------|--------------------------|--------------------|--------|----------|------------|
| 1              | Hor.                | 2                        | 100% water         | 260    | .492     | 519        |
| 2              | Hor.                | 0.075                    | do                 | 260    | .573     | 558        |
| 3              | Hor.                | 2                        | 90% water, 10% DMF | 270    | .511     | 491        |
| 4              | Hor.                | 0.075                    | do                 | 215    | .570     | 575        |
| 5              | Hor.                | 2                        | 75% water, 25% DMF | 279    | .760     | 516        |
| 6              | Hor.                | 0.075                    | do                 | 282    | .668     | 592        |
| 7              | Vertical            | 0.075                    | do                 | 265    | .770     | 630        |

tion may be extruded through a single orifice or a plurality of orifices in the spinneret to form a filament or bundle of filaments. The extruded streams of polymer are directed through the coagulating liquid for a predetermined minimum distance to cause the solution to coagulate, the distance being from about 0.5 to 3.0 inches. The filaments 6 are withdrawn by positively driven roller 7.

The linear, segmented polyurethane polymers which are suitable for use in the improved wet spinning process of the invention include any and all of the well known linear, segmented polyurethane polymer compositions of the prior art sometimes referred to as spandex type elastomers. Such polyurethane compositions are typified by those disclosed in U.S. Patents 2,957,852; 2,929,804; and 3,097,192 and are generally described as comprising urea segments linked to polyester or polyether segments through urethane groups.

The process of this invention represents an improvement in the wet spun preparation of elastic fibers and filaments from linear, segmented polyurethane polymers in several respects. Consistently reproducible elongations in excess of 500 percent are possible using the process of the invention. Tenacities greater than 0.7 gram per denier, more uniform yarn and faster spinning speeds of up to 200 ft./min. are also possible. The permanent set of elastic filaments produced by the process of the invention ranges from 26 to 28 percent with high elastic recovery and stress retention values of more than commercially acceptable ranges. A wide range of solvents may also be used in the process of the invention.

The elastic fibers and filaments of the invention are useful in a variety of applications such as in fabrics, women's lingerie, support hose and similar textile end uses.

The invention is further illustrated by the following examples in which all parts and percents are by weight unless otherwise indicated. In the examples the cited physical properties were measured on the Instron Tester, Model TM. "Tenacity" measurements are expressed in grams per denier (g.p.d.), the fibers being stretched at a rate of 1000 percent per minute. "Elongation" is the percent

49 50 55 extension of the fibers at the breaking point. "Stress retention" is the percent elasticity retained after 300% extension and 80% recovery of the 2nd cycle stretch.

#### EXAMPLE II

A 300-part portion by weight of poly(tetramethylene glycol) of molecular weight 2,600 was reacted with 58.5 parts of 4,4'-methylenediphenyl diisocyanate in 197 parts dimethylformamide solvent for one hour. The resulting prepolymer was added to a solution of 0.948 gram of hydrazine hydrate in 1844 parts dimethylformamide solvent to give a spinning dope of 15% solids. This spinning dope was extruded both horizontally and vertically through a spinneret 15 holes of 6 mil diameter into a bath containing 75% water and 25% dimethylformamide at 70° C. The residence time of the fiber in the spin bath was two seconds when spun horizontally and 0.075 second when spun vertically. The fiber was washed, dried and taken up at a speed of 100 feet a minute. Properties of this fiber are given by Table II and show the improvement obtained when using vertical short residence over horizontal long residence time.

#### EXAMPLE III

A 300 part portion by weight of a polycaprolactone, consisting of 80% polycaprolactone and 20% poly(methylcaprolactone), of molecular weight 1,850 is reacted with 85.1 parts of 4,4'-methylenediphenyl diisocyanate in 210 parts dimethylformamide for one hour. The prepolymer is then added to a solution of 5.9 grams of carbodihydrazide in 2009 parts dimethylformamide to give a spinning dope. This spinning dope is then extruded using the conditions described in Example II. The properties of these fibers are also given in Table II showing the improvement in vertical short residence over horizontal long residence time spinning.

#### EXAMPLE IV

A 400-part portion by weight of a polyester, composed of 80% polyethylene adipate and 20% polypropylene adipate, of molecular weight 1,690 was reacted with 124 parts of 4,4'-methylenediphenyl diisocyanate in 286 parts dimethylformamide solvent for 2 hours. This prepolymer was added to a solution of 10 parts of m-xylylene diamine

in 2740 parts of dimethylformamide to give a spinning dope. This spinning dope was extruded using the conditions described in Example II. The properties of the resulting fibers are given in Table II.

TABLE II

| Example | Spinneret | Spin Bath Time (sec.) | Denier | Elongation, Percent | Percent Stress Retention |
|---------|-----------|-----------------------|--------|---------------------|--------------------------|
| I       | Hor.      | 2.000                 | 279    | 516                 | 18.9                     |
|         | Vertical  | 0.075                 | 265    | 630                 | 24.9                     |
| II      | Hor.      | 2.000                 | 228    | 580                 | 10.7                     |
|         | Vertical  | 0.075                 | 265    | 631                 | 12.7                     |
| III     | Hor.      | 2.000                 | 263    | 501                 | 11.9                     |
|         | Vertical  | 0.075                 | 290    | 524                 | 15.2                     |
| IV      | Hor.      | 2.000                 | 330    | 527                 | 11.4                     |
|         | Vertical  | 0.075                 | 205    | 600                 | 17.2                     |

## EXAMPLE V

This example illustrates the fact that increasing the spinning speed from 100 ft./min. to 170 ft./min. may be accomplished without any deterioration of fiber properties.

The polymer composition of Example I was extruded using a 0.075-second vertical immersion method at spinning speeds of 100 and 170 ft./min. The yarn properties are shown below.

|                                           | 100 ft./min. | 170 ft./min. |
|-------------------------------------------|--------------|--------------|
| Tenacity                                  | 1.07         | 0.94         |
| Elongation                                | 588          | 560          |
| Percent Stress Retained 80%, 2nd Recovery | 22.1         | 21.9         |

## EXAMPLE VI

The permanent set of fibers prepared from the polymer composition of Example I is improved when wet spun vertically as shown by the following data.

Percent set (20 sample average): 2 secs. horizontal, 35; 35 0.075 sec. vertical, 28.

Similar improvement in elongation, tenacity, modulus, permanent set, stress retention and spinning speeds will be noted when other linear, segmented polyurethane compositions are wet spun according to the process of the invention.

The foregoing detailed description has been given for clearness of understanding only, and unnecessary limitations are not to be construed therefrom. The invention is not to be limited to the exact details shown and described since obvious modifications will occur to those skilled in the art, and any departure from the description herein that conforms to the present invention is intended to be included within the scope of the claims.

We claim:

1. In the process for wet spinning of linear, segmented polyurethane polymers to produce elastomeric polyurethane fibers and filaments, the improvement consisting of advancing the filaments as they are coagulated upwardly through the coagulating bath a distance of up to about 3.0 inches at a rate of withdrawal which will result in the filaments remaining in the coagulating bath for a period of time of up to about 0.2 second.

2. In the process for wet spinning of linear, segmented polyurethane polymers to produce elastomeric polyurethane fibers and filaments, the improvement consisting of advancing the filaments as they are coagulated upwardly

through the coagulating bath a distance of from 0.5 to 3.0 inches at a rate of withdrawal which will result in the filaments remaining in the coagulating bath for a period of time of from about 0.075 to 0.1 second.

3. In the process for wet spinning of linear, segmented polyurethane polymers to produce elastomeric polyurethane fibers and filaments, the improvement consisting of advancing the filaments as they are coagulated upwardly through the coagulating bath so that the filaments will move essentially vertically with respect to the surface of the coagulating bath liquid for a distance of from 1.5 to 2.0 inches at a rate of withdrawal which will result in the filaments remaining in the coagulating bath for a period of time of from about 0.075 to 0.1 second.

25 4. In the process for wet spinning of linear, segmented polyurethane polymers to produce elastomeric polyurethane fibers and filaments, the improvement consisting of advancing the filaments as they are coagulated upwardly through the coagulating bath consisting essentially of water and from 1 to 40 percent of dimethylformamide so that the filaments will move essentially vertically with respect to the surface of the coagulating bath liquid for a distance of from 1.5 to 2.0 inches at a rate of withdrawal which will result in the filaments remaining in the coagulating bath for a period of time of from about 0.075 to 0.1 second.

30 5. In the process for wet spinning of linear, segmented polyurethane polymers to produce elastomeric polyurethane fibers and filaments, the improvement consisting of advancing the filaments as they are coagulated upwardly through the coagulating bath consisting essentially of water and from 1 to 40 percent of dimethylacetamide so that the filaments will move essentially vertically with respect to the surface of the coagulating bath liquid for a distance of from 1.5 to 2.0 inches at a rate of withdrawal which will result in the filaments remaining in the coagulating bath for a period of time of from about 0.075 to 0.1 second.

## 50 References Cited

## UNITED STATES PATENTS

- 3,036,878 5/1962 Polansky ----- 264-178  
3,037,240 6/1962 Stoy ----- 264-182

## 55 OTHER REFERENCES

Hill, Rowland, editor, "Fibres From Synthetic Polymers," 1953, Elsevier Publishing Company (Amsterdam-Houston-New York-London), pp. 379-388 and 461.

60 JAMES A. SEIDLECK, Primary Examiner.

ALEXANDER H. BRODMERKEL, Examiner.

H. MINTZ, Assistant Examiner.

UNITED STATES PATENT OFFICE  
CERTIFICATE OF CORRECTION

Patent No. 3,388,200

June 11, 1968

Charles E. Jackson et al

It is certified that error appears in the above identified patent and that said Letters Patent are hereby corrected as shown below:

Column 2, line 7, "2,955,07;" should read -- 2,955,017; --. Column 4, line 18, "varied from 2 to 0.75 seconds." should read varied from 2 to 0.075 seconds. --.

Signed and sealed this 10th day of March 1970.

(SEAL)

Attest:

Edward M. Fletcher, Jr.

Attesting Officer

WILLIAM E. SCHUYLER, JR.

Commissioner of Patents